

# United States Patent [19]

Yaffe et al.

[11]

4,189,388

[45]

Feb. 19, 1980

[54] SYNTHETIC AIRCRAFT TURBINE OIL

[75] Inventors: Roberta Yaffe, Glenham; Russell R. Reinhard, Hopewell Junction, both of N.Y.

[73] Assignee: Texaco Inc., White Plains, N.Y.

[21] Appl. No.: 864,984

[22] Filed: Dec. 27, 1977

[51] Int. Cl.<sup>2</sup> ..... C10M 1/48

[52] U.S. Cl. ..... 252/46.7; 252/47.5;  
252/48.6; 252/56 S

[58] Field of Search ..... 252/46.7, 47.5, 48.6,  
252/56 S

[56] References Cited

U.S. PATENT DOCUMENTS

2,603,653 7/1952 Kosmin et al. ..... 252/48.6 X  
3,360,465 12/1967 Warman ..... 252/56 S

|           |         |                     |            |
|-----------|---------|---------------------|------------|
| 3,505,225 | 4/1970  | Wheeler .....       | 252/47.5   |
| 3,779,919 | 12/1973 | Patmore et al. .... | 252/47.5 X |
| 4,076,639 | 2/1978  | Bridger et al. .... | 252/47.5   |
| 4,088,587 | 5/1978  | Lowe .....          | 252/48.6 X |
| 4,097,386 | 6/1978  | Lowe .....          | 252/48.6 X |

Primary Examiner—Andrew Metz  
Attorney, Agent, or Firm—Robert A. Kulason; Carl G. Ries; James F. Young

[57]

## ABSTRACT

Synthetic lubricating oil composition having improved oxidation stability comprising a major portion of an aliphatic ester base oil having lubricating properties formed by the reaction of pentaerythritol and an organic monocarboxylic acid and containing a phenyl-naphthylamine, a dialkyldiphenylamine, a polyhydroxy anthraquinone, a hydrocarbyl phosphate ester and a thioacid derivative compound as hereinafter described.

9 Claims, No Drawings

## SYNTHETIC AIRCRAFT TURBINE OIL

## BACKGROUND OF THE INVENTION

## Field of the Invention

This invention is concerned with a pentaerythritol ester base lubricating oil composition for a gas turbine engine. Gas turbine engines are operated under a wide range of temperature conditions. The lubricant must be fluid at extremely low temperatures and at the same time retain its lubricating properties in an engine which produces internal operating temperatures at 450°-550° F. or above. The lubricant is subjected to severe oxidation stresses under the high running temperatures encountered in such engines.

Ester base lubricating oil compositions prepared from pentaerythritol and a mixture of fatty acids and containing selected additive combinations are well known. These lubricants are functional over a wide temperature range and exhibit good thermal and oxidative stability. The search for a still more effective, long lived ester base lubricant composition, however, is a major goal of lubricant manufacturers. In addition, more advanced gas turbine engines currently being developed and tested will put higher stresses on the lubricant composition and are projected to require improved lubricant compositions.

## SUMMARY OF THE INVENTION

The synthetic lubricating oil composition of the invention comprises a major portion of an aliphatic ester base oil containing a phenyl naphthylamine, a dialkyldiphenylamine, a polyhydroxy anthraquinone, a hydrocarbyl phosphate ester and a thioacid derivative as hereinafter described. More specifically, the lubricating oil composition of the invention comprises a major portion of an aliphatic ester base oil formed from the reaction of pentaerythritol and an organic monocarboxylic acid having from about 2 to 18 carbon atoms per molecule containing:

(a) from about 0.3 to 5 percent by weight of the lubricating oil composition of phenyl naphthylamine or an alkyl or alkaryl derivative of phenyl naphthylamines in which the alkyl radicals contain from 4 to 12 carbon atoms,

(b) from about 0.3 to 5 percent by weight of a dialkyl-diphenylamine in which the alkyl radicals contain from 4 to 12 carbon atoms,

(c) from about 0.001 to 1 percent by weight of a polyhydroxyanthraquinone,

(d) from about 0.25 to 10 percent by weight of a hydrocarbyl phosphate ester in which said hydrocarbyl radical containing an aryl ring and has from about 6 to 18 carbon atoms, and

(e) from about 0.01 to 5.0 percent by weight of a thioacid derivative compound as hereinafter described.

The lubricating oil composition of the invention provides substantial improvements in oxidative stability, particularly excellent control of acidity and viscosity increase under severe oxidizing conditions.

## DETAILED DESCRIPTION

The base fluid component of the composition of the invention is an ester-base fluid prepared from pentaerythritol and a mixture of hydrocarbyl monocarboxylic acids. Polypentaerythritols, such as dipentaery-

thritol, tripentaerythritol and tetrapentaerythritol can also be employed in the reaction to prepare the base oil.

The hydrocarbon monocarboxylic acids which are used to form the ester-base fluid include the straight-chain and branched-chain aliphatic acids, as well as mixtures of these acids. The acids employed have from about 2 to 18 carbon atoms per molecule, and preferably from about 5 to 10 carbon atoms. Examples of suitable acids are acetic, propionic, butyric, valeric, isovaleric, caproic, decanoic, dodecanoic, tertiarybutylacetic and 2-ethylhexanoic acid, including mixtures.

In general, the acids are reacted in proportions leading to a completely esterified pentaerythritol or poly-pentaerythritol with the preferred ester bases being the pentaerythritol tetraesters. Examples of such commercially available tetraesters include pentaerythritol tetrapropionate, which is prepared from purified pentaerythritol and crude caproic acid containing other C<sub>5</sub>-10 monobasic acids. Another suitable tetraester is prepared from a technical grade pentaerythritol and a mixture of acids comprising 38 percent valeric, 13 percent 2-methyl pentanoic, 32 percent octanoic and 17 percent pelargonic acids, by weight.

The ester base fluid comprises the major portion of the fully formulated synthetic ester base lubricating oil composition. In general, this ester base fluid is present in concentrations from about 90 to 98 percent of the composition, by weight.

The essential alkyl or alkaryl phenyl naphthylamine component of the invention is represented by the formula:



in which R may be H or is an alkyl radical containing from about 4 to 12 carbon atoms or an alkaryl radical containing from 7 to 12 carbon atoms. This radical can be straight or branched chain alkyl radical with the tertiary alkyl structure being preferred or it can be an alkaryl radical.

Specific effective compounds of this class include  $\alpha$  or  $\beta$  phenylnaphthylamine, N-(para-tertiary-octyl-phenyl)- $\alpha$  or  $\beta$ -naphthylamine, N-(4-cumylphenyl)  $\alpha$  or  $\beta$ -naphthylamine and the corresponding parateriary-dodecylphenyl and parateriary-butylphenyl alpha-and beta-naphthylamines. The preferred naphthylamines are those in which R is H or a tertiary alkyl radical having from 6 to 10 carbon atoms therein. The preferred concentration of this component is from about 0.5 to 2.5 percent by weight.

Another essential component of the lubricating oil composition of the invention is a dialkyldiphenylamine. These compounds are represented by the formula:



in which R is an alkyl radical having from about 4 to 12 carbon atoms. Suitable alkylamines include dioctyldiphenylamine, didecyldiphenylamine, didodecyldiphenylamine, dihexyldiphenylamine and similar compounds. Dioctyldiphenylamine is the preferred com-

pound and the preferred concentration is from 0.5 to 2.0 percent by weight.

The essential metal deactivator of the lubricating oil composition of the invention is a polyhydroxyanthraquinone. Suitable compounds in this class are the dihydroxyanthraquinones such as 1,4-dihydroxyanthraquinone and 1,5-dihydroxyanthraquinone and the higher polyhydroxyanthraquinones such as 1,2,5,8 tetrahydroxyanthraquinone. The preferred concentration of this component is from about 0.05 to 0.15 weight percent.

Another component of the lubricating oil composition of the invention is a hydrocarbyl phosphate ester, more specifically a trihydrocarbyl phosphate in which the hydrocarbyl radical is an aryl or alkaryl, radical or mixture thereof containing from 6 to 18 carbon atoms and preferably from 6 to 12 carbon atoms. Effective specific compounds include tricresylphosphate. These compounds are preferably in the lubricating oil composition in a concentration ranging from about 0.5 to 5 wt. %.

Another essential component of the lubricating oil composition is a thioacid derivative compound represented by the formula



where R is a straight chain or branched chain alkyl radical containing from about 4 to 20 carbon atoms therein, X is either O or NH, and n is 1 or 2.

Representative thioacid derivative compounds include the dialkylthio diglycolates, dialkylthio dipropionates dialkylthio diglycolamides and dialkylthio dipropionamides wherein the alkyl substituent is a straight or branched chain alkyl radical such as a butyl, pentyl, hexyl, heptyl, octyl, nonyl, decyl, undecyl, dodecyl, tridecyl, tetradecyl, pentadecyl, hexadecyl and so forth.

This constituent is present in the lubricating oil composition in an amount of from about 0.01 to about 5.0% preferably in a concentration range of from about 0.5 to about 2.5 by weight.

The novel lubricating oil compositions of the present invention exhibit improved oxidation stability particularly excellent control of acidity and viscosity increase under severe oxidizing conditions.

The ester base oil employed in preparing the lubricating oil composition of the invention comprised pentaerythritol containing a minor amount of dipentaerythritol esterified with a mixture of fatty acids. It consisted of technical grade pentaerythritol ester made from a mixture of carboxylic acids consisting of (mole %):

|                  |         |
|------------------|---------|
| i-C <sub>5</sub> | 8 ± 3%  |
| n-C <sub>5</sub> | 23 ± 5% |
| n-C <sub>6</sub> | 20 ± 5% |
| n-C <sub>7</sub> | 27 ± 5% |
| n-C <sub>8</sub> | 7 ± 3%  |
| n-C <sub>9</sub> | 16 ± 3% |

This ester base oil had the following properties:

Viscosity, cs at 210° F.

(5.01)

-continued

|   |                          |        |
|---|--------------------------|--------|
| 5 | Viscosity, cs at 100° F. | (25.6) |
|   | Viscosity, cs at -40° F. | (7005) |
|   | Viscosity Index          | (140)  |
|   | Flash, °F.               | (515)  |

The above ester oil was blended with all of the prescribed essential additives with the exception of the thioacid derivative to form a Base Fluid. Based on a fully formulated lubricant composition, the Base Fluid consisted of about 95.4 weight percent of the ester base oil described above with 1.5 weight percent of t-octyl-phenyl- $\alpha$ -naphthylamine, 1.0 weight percent of dioctyl-diphenylamine, 2.0 weight percent of tricresylphosphate and 0.1 weight percent of quinizarin.

The oxidation-stability of the lubricants of the invention as compared to the Base Fluid was determined in the Rolls Royce (RR 1001) Oxidation Test. (D. Eng. R.D. 2497 Supplement Method No. 12). The results are set forth in the following Table.

TABLE I

| 25 | Rolls Royce (RR 1001) Oxidation Test<br>Dilaurylthio-Dipropionate |                     |                |                     |
|----|-------------------------------------------------------------------|---------------------|----------------|---------------------|
|    | Conditions                                                        |                     |                |                     |
|    | 230° C./40 Hrs.                                                   |                     | 260° C./6 Hrs. |                     |
|    | Base Fluid                                                        | 0.05 Wt. % Additive | Base Fluid     | 0.10 Wt. % Additive |
| 30 | % Viscosity Change<br>at 100° F.                                  | 253                 | 171            | 80.6                |
|    | Total Acid Number<br>Change                                       | 6.02                | 5.96           | 5.28                |
|    |                                                                   |                     |                | 3.94                |

35 The data in Table I above show that the oxidative stability of the lubricating oil compositions of the present invention containing the dialkylthio-dipropionate species are significantly improved in comparison to the Base Fluid.

40 In comparison to the Base Fluid, the dialkylthio dipropionate species showed a reduction in Viscosity Increase of about 32.4% at 0.05% wt. concentration and a reduction of 25% at 0.1 wt. % concentration.

45 The Total Acid Number Increase change at 0.05 and 0.1 wt. % concentrations respectively were 1% and 25.4% less than those of the Base Fluid.

50 The lubricating oil compositions containing the dialkylthio-dipropionate species were further evaluated at 0.1 wt. concentration in the Pratt and Whitney Aircraft Specification PWA-521C Oxidation-Corrosion Test 425° F./48 HRS. and the Navy MIL-L-23699B Specification 400° F./72 HRS. Oxidation Corrosion Test and were found to satisfy completely these specification requirements.

55 The following Table II illustrates that the thioacid derivatives can be used as a replacement for the dialkyl diphenylamine constituent in the Base Fluid.

TABLE II

| 60 | Rolls Royce (RR 1001) Oxidation Test<br>Dilaurylthio-Dipropionate |                           |      |
|----|-------------------------------------------------------------------|---------------------------|------|
|    | BASE Fluid +<br>1.0 Wt. %<br>Additive                             |                           |      |
|    | In Place Of The Dialkyl<br>Diphenylamine Constituent              |                           |      |
| 65 | Base Fluid                                                        | Diphenylamine Constituent |      |
|    | % Viscosity Change<br>at 100° F.                                  | 95.6                      | 46.1 |
|    | Total Acid                                                        |                           |      |

TABLE II-continued

| Rolls Royce (RR 1001) Oxidation Test<br>Dilaurylthio-Dipropionate |                                       | In Place Of The Dialkyl<br>Diphenylamine Constituent |
|-------------------------------------------------------------------|---------------------------------------|------------------------------------------------------|
| Base Fluid                                                        | BASE Fluid +<br>1.0 Wt. %<br>Additive |                                                      |
| Number Change                                                     | 4.23                                  | 3.57                                                 |

The lubricating oil compositions containing the dialkylthio-dipropionate species were further evaluated at 1.0 wt. % concentration in the Pratt and Whitney Aircraft Specification PWA-521C Oxidation-Corrosion Test 425° F./48 HRS. and the Navy MIL-L-23699B Specification 400° F./72 HRS. Oxidation Corrosion Test and were found to satisfy completely these specification requirements.

The data in the above Table II further illustrate that the thioacid derivative compounds of the present invention, particularly the dialkylthio-dipropionate species, can be used as a replacement for either of the major antioxidant components of the Base Fluid, i.e. the naphthylamine or the phenylamine component, and thereby attain excellent results.

At 1.0 wt. % concentration, as replacement for the dialkyl diphenylamine constituent in the Base Fluid the dialkylthio-dipropionate species of the invention showed a 51.2% decrease in Viscosity Increase in comparison to the Base Fluid.

The Total Acid Number Increase change at 1.0 wt. % concentration was 15.6% less than that of the Base Fluid.

TABLE III

| Rolls Royce (RR 1001) Oxidation Test<br>260° C./6 Hrs. |            |                                       |            |                                       |
|--------------------------------------------------------|------------|---------------------------------------|------------|---------------------------------------|
| N,N'-Di(Beta-Undecyl) Thiodipropionamide               |            |                                       |            |                                       |
|                                                        | Base Fluid | Base Fluid +<br>0.1 Wt. %<br>Additive | Base Fluid | Base Fluid +<br>0.5 Wt. %<br>Additive |
| % Viscosity<br>Change at 100° F.                       | 96.7       | 56.5                                  | 96.7       | 35.2                                  |
| Total Acid<br>Number Change                            | 4.09       | 3.00                                  | 4.09       | 3.23                                  |

The data in the Table III above show that the oxidative stability of the lubricating oil compositions containing the amide species are significantly improved in comparison to the Base Fluid.

In comparison to the Base Fluid, the composition showed a reduction in Viscosity Increase of about 41.6% at 0.1% wt. concentration and 66.6 at 0.5 wt. % concentration.

At 0.1 wt. % concentration, the composition showed a 26.7% decrease in Total Acid Number Change and a 55 decrease of 26.6% at 0.5 wt. %.

The lubricating oil composition containing the amide species of the invention at 0.1 wt. % concentration was further evaluated in the Navy MIL-L-23699B Specifi-

cation 400° F./72 HRS. Oxidation Corrosion Test and was found to satisfy these specification requirements.

Obviously, many modifications and variations of the invention as hereinbefore set forth may be made without departing from the spirit and scope thereof and therefore only such limitations should be imposed as are indicated in the appended claims.

We claim:

1. A synthetic lubricating oil composition consisting of a major portion of an aliphatic ester base oil having lubricating properties formed from the reaction of pentaerythritol or a polypentaerythritol or trimethylolpropane and an organic monocarboxylic acid having from about 2 to 18 carbon atoms per molecule and:

(a) from about 0.3 to 5 percent by weight of the lubricating oil composition of a phenylnaphthylamine or an alkyl or alkaryl phenyl naphthylamine in which the alkyl radical has from 4 to 12 carbon atoms,

(b) from about 0.3 to 5 percent by weight of a dialkyl-diphenylamine in which the alkyl radicals have from 4 to 12 carbon atoms,

(c) from about 0.01 to 0.5 percent by weight of a polyhydroxy-substituted anthraquinone,

(d) from about 0.25 to 10 percent by weight of a hydrocarbyl phosphate ester in which said hydrocarbyl radical contains an aryl ring and contains from about 6 to 18 carbon atoms, and

(e) from about 0.01 to about 5.0 percent by weight of a N,N'-dialkylthio dipropionamide wherein each alkyl radical is a straight or branched chain alkyl radical containing from 4 to 20 carbon atoms therein.

2. A lubricating oil composition as claimed in claim 1 wherein said N,N'-dialkylthio dipropionamide is N,N'-di(betaundecyl) thiodipropionamide.

3. A lubricating oil composition as claimed in claim 1 containing from about 0.05 to about 2.5 percent by weight of said thioacid derivative.

4. A lubricating oil composition as claimed in claim 1 wherein the naphthylamine is octylphenyl-alpha-or-beta-naphthylamine.

5. A lubricating oil composition as claimed in claim 1 containing from about 0.5 to 2.0 percent of a dialkyldiphenylamine, by weight.

6. A lubricating oil composition as claimed in claim 1 containing from about 0.01 to 0.5 percent of said polyhydroxy-substituted anthraquinone, by weight.

7. A lubricating oil composition as claimed in claim 6 wherein the polyhydroxy-substituted anthraquinone is 1,4-dihydroxyanthraquinone.

8. A lubricating oil composition as claimed in claim 1 containing from about 0.5 to 5 percent of a hydrocarbyl phosphate ester, by weight.

9. A lubricating oil composition as claimed in claim 1 wherein the aliphatic ester base oil is present in a concentration of from about 90 to 98 percent of the composition, by weight.

\* \* \* \* \*